

W. GENEST & H. STÖSSEL.  
PLATE FOR DEADENING VIBRATION AND SOUND.  
APPLICATION FILED JULY 14, 1909.

971,369.

Patented Sept. 27, 1910.

2 SHEETS—SHEET 1.

Fig. 1.



Fig. 2.



WITNESSES:

C. J. Patches  
Galley & Yuditz.

INVENTORS:

Werner Genest  
Hugo Stössel

Br. D. P. A. Schuck: ATTORNEY.

W. GENEST & H. STÖSSEL.  
PLATE FOR DEADENING VIBRATION AND SOUND.  
APPLICATION FILED JULY 14, 1909.

971,369.

Patented Sept. 27, 1910.

2 SHEETS-SHEET 2.

Fig.3.



Fig.4.



Fig.5.



Fig.6.



WITNESSES:

C. J. Thatchin  
Sally & Judyky.

INVENTORS:

Werner Genest  
Hugo Stössel

BY *Frank D. Schueler* ATTORNEY.

# UNITED STATES PATENT OFFICE.

WERNER GENEST, OF GROSS-LICHTERFELDE, AND HUGO STÖSSEL, OF WESTEND,  
GERMANY.

## PLATE FOR DEADENING VIBRATION AND SOUND.

971,369.

Specification of Letters Patent. Patented Sept. 27, 1910.

Application filed July 14, 1909. Serial No. 507,664.

*To all whom it may concern:*

Be it known that we, WERNER GENEST and HUGO STÖSSEL, both subjects of the German Emperor, and residents, respectively, of 5 Gross-Lichterfelde and Westend, in the Kingdom of Prussia, German Empire, have invented new and useful Improvements in Plates for Deadening Vibration and Sound, of which the following is a full, clear, and 10 exact specification.

Our invention relates to cork sheets for deadening vibration and sound.

For preventing or deadening the transmission of sound and vibration in machinery 15 plants, railways, and the like, sheets of cork are used as insulation. The sheets are generally placed between the machine, engine or the like and its foundation, but they may also be arranged at the sides of the machine 20 or in any other suitable position, according to the direction in which transmission that is to be prevented is likely to occur. Such sheets are generally made of natural cork cut into strips of suitable size and made into 25 sheets by joining a number of these strips together, the whole being confined by an iron band or hoop around the periphery of the sheet. A sheet made up in this way is apt to lose its shape and to become less efficient 30 because the weight or pressure of the machine causes the cork to expand laterally and either ruptures or distorts the iron band or hoop.

Now a primary object of our invention is 35 to provide a cork sheet or plate which is stronger and more durable than those known heretofore. This object is attained by providing in the sheet or plate a number of cross-ties or reinforcing bars; for instance 40 the frame-work of the plate, instead of being merely a confining hoop is a grid or grating the transverse bars of which act as ties for the surrounding hoop or band.

Care must be taken that there is no metal- 45 lic conduction between the foundation and the machine. The inserted bands or rods must therefore be of less depth than the thickness of the cork.

In order that our invention may be clearly 50 understood we will now explain the same with reference to the accompanying drawings in which one embodiment is represented by way of example.

In said drawings, Figure 1 is a plan, 55 partly in horizontal section of a cork plate

or sheet made, according to our invention; Fig. 2 is a side view of the same, partly in vertical section; Fig. 3 is a side elevation of a metal strip inserted between the cork strips; Fig. 4 is a section of this strip, where- 60 as Fig. 5 is a section through a sheet made up of the separate strips, and Fig. 6 is a side elevation of two cork strips, one of which is broken away.

Referring to the drawings, *a* is a hoop 65 made of an iron band or the like provided with cross-ties or reinforcing bars *b* forming a grating and firmly connected with the hoop *a*, the bars *b* also being preferably made of iron bands or the like. The compartments so formed are filled with cork by cutting the natural cork into strips *c* of suitable size and putting these strips, in the manner shown in the drawings, into the compartments formed by the hoop *a* and 70 bars *b*. The cork strips are made of such thickness as to project above and below the hoop *a* and bars *b* as shown in Fig. 2. Thus no metallic contact can take place between the foundation and the engine or the like 75 placed on the cork plate. The cork strips being in immediate contact with the inner bars *b* are preferably laterally cut away, as shown in Fig. 2, so as to overlap and cover the bars *b* from above and from below. 80 These cork plates are preferably impregnated with some liquid which is not likely to dry under the conditions in question in each instance. The reason for this is that when a cork plate not treated in this manner 85 is used to insulate the foundation of a machine in a heated room, the cork in time loses some of its water and become brittle. Apart from the fact that this affects the 90 life of the plate, brittle cork will transmit vibrations and sounds considerably better 95 than cork which, owing to a certain amount of liquid contained therein, is elastic. Notwithstanding, therefore, that vibration and noise may be satisfactorily deadened at first, 100 the efficiency of the plate will gradually decrease under conditions entailing the drying of the cork. In order to prevent the cork from becoming brittle, it is impregnated, before being put in place, with practically 105 non-drying liquids such as tar oils, *e. g.* carbolic oil having a boiling point 230°-250° C., creosote oil or heavy oils having a boiling point 250°-280° C., crude petroleum, heavy petroleum or the like. The 110

impregnation can be effected by dipping either the separate strips of which the plate is made or the completed plate into a vessel which has been filled with the impregnating liquid. If necessary the impregnation can be effected at an increased temperature or even at increased or decreased pressure. Under general circumstances it is sufficient to immerse the cork in the liquid for a few hours without diminishing the pressure. It should be pointed out that many sorts of tar, asphalt or the like which have been used as a binding medium for producing cork plates from residues, are not suitable for saturating cork for the purpose of this invention since they harden comparatively quickly, and would thus form a most unsuitable insulating material for deadening vibrations and noises.

It is preferable that the impregnating fluid should also have antiseptic properties, which is the case with most of the liquids named; if the liquid is devoid of such property an antiseptic may be separately used.

In order to prevent the separate cork strips from relative movement or from falling out, insertions may be arranged between the strips, friction between which and the strips prevents relative movement. For instance, strips of sheet metal with roughened surfaces may be used. The teeth or roughnesses enter the cork strips and so prevent them from shifting.

In Figs. 3, 4, 5 and 6, *d* are the teeth on the one side, *e* those on the other side of the metal strip. Fig. 6 shows the strip bent twice at an angle so as to form a connection between the ends of two strips.

The form and number of the teeth depends entirely on the stress likely to cause the cork strips to shift. Instead of metal strips, bands or strips of other suitable material such as sand-paper sanded on both faces, may be used. When metal or like strips are

used, care must be taken that they are not 45 as deep as the cork strips, in order that when strong pressure is exerted on the finished plate the metal or like strips do not project beyond the compressed cork and thus form a conductor for vibrations and 50 sounds.

If desired the sheets may be perforated or may contain cavities to increase their elasticity.

We claim:—

1. In a plate for deadening vibration and sound, the combination of a metal frame having transverse reinforcing bars, and a plurality of sheets of cork held in said frame, each sheet of cork comprising a plurality of strips of cork and roughened insertions placed between the same. 55

2. In a plate for deadening vibration and sound, the combination of a metal frame having transverse reinforcing bars, and a 65 plurality of sheets of cork held in said frame, each sheet of cork comprising a plurality of strips of cork and metal strips, provided with oppositely disposed spurs or teeth, placed between the same. 70

3. In a plate for deadening vibration and sound, the combination of a metal frame having transverse reinforcing bars, and a plurality of sheets of cork held in said frame, each sheet of cork comprising a plurality of strips of cork and metal strips, of a depth less than that of the cork strips and provided with oppositely disposed spurs or teeth, placed between the same. 75

In testimony, that we claim the foregoing 80 as our invention, we have signed our names in presence of two subscribing witnesses.

WERNER GENEST.

HUGO STÖSEL.

Witnesses:

WOLDEMAR HAUPT,  
HENRY HASPER.